

## UNITED STATES PATENT OFFICE

1,996,039

METHOD FOR WORKING READY DRESSED  
AND TANNED PELTS

Philipp Burger, Berlin, Germany

No Drawing. Application May 19, 1934, Serial  
No. 726,574. In Germany May 20, 1933

3 Claims. (Cl. 149—28)

This invention relates to a method, according to which ready dressed and tanned pelts can be worked to form a novel product which is suitable for making articles of clothing, for example coats, but particularly also articles of use such as handbags or the like. According to the invention even inferior quality pelts, for example skins which moult and were hitherto useless can be improved without detrimentally affecting the durability and good appearance of the new product.

According to the invention the hair side of the pelt is painted with adhesive solutions, wherefrom the hairs are brushed against the skin with a brush, roller or the like. Different patterns of a pelt are produced according to the manner in which the hairs bear against the skin. By this treatment the skin itself is strengthened, and the hairs, which perhaps from nature do not even hold tightly, are secured in such a manner that a very durable product is produced, seeing that the hairs united with the skin also considerably strengthen the skin. The appearance of this product can be varied by the treatment, also as regards its gloss, color and the like.

The application of the adhesive solutions is effected, for example, in the following manner:—

Pour 10 parts by weight of very finely pulverized French colophony into 100 parts of water and also 2 parts of caustic soda; boil the mixture until the substances are dissolved and then allow the solution to cool to 50° C. This resin soap is applied onto the hair side of the skin in the direction in which the hairs have grown and well distributed thereon. A second solution is then formed by boiling 4 parts of ferrous sulphate in 100 parts of water, which solution is cooled to 50° C. and rapidly distributed under pressure over the soap coating, likewise on the hair side of the skin in the direction of the hairs, so that a sticky, tough layer of iron resin soap is formed over the hair and is allowed to dry with the skin in flat condition. The skin may if desired be lacquered on the day following the drying with a black cellulose lacquer by means of a brush and allowed to dry, this requiring a few hours, according to the kind of lacquer employed, whereupon the skin is coated with a colorless cellulose lacquer.

The method is simpler and cheaper with layers of kinds of glue or glue substances, such as gelatine or isinglass dissolved by swelling in water

and rendered waterproof and resistant after drying by admixtures of bichromates. These layers stick down the hairs.

*Example.*—10 grs. of pearl glue are swelled over night in 50 cub. cms. of water to which 5 cub. cms. of chemically pure 80% lactic acid have been added, then stirred and allowed to stand four days in the light, whereupon the glue is dissolved by stirring. The solution has a clear acid reaction on litmus. 10 grs. of powdered sugar, 10

10 cub. cms. industrial glycerine, 5 grs. crystallized logwood extract and 5 cub. cms. of industrially pure castor oil are separately poured into 50 cub. cms. of water and shaken, whereupon the mixture is boiled well for ten minutes in a water bath to dissolve the logwood extract, and thereupon 1 gr. of chrome leather black dye is dissolved therein by again boiling for five minutes. Shake the solution, allow to cool to 30° C. and gradually add it to the first glue solution stirring 20 the whole, so that the mixture now contains the dyes and the organic substances, in order to subsequently reduce the tanning bichromate or the chromic acid. The glue sticks down the hairs in wet condition, but is water fast after drying. 25 The addition of castor oil makes the leather of the felt softer because the glue layer alone hardens too much—5 grs. of ammonium bichromate are now dissolved in 50 cub. cms. water by shaking or heating, whereupon the solution is allowed 30 to cool to 30° C. and carefully added in doses to the above mentioned glue solution, stirring the while.

It is advisable to sew together the ready dressed and tanned pelts to form long and large webs before the treatment according to the invention is applied so that continuous large surfaces of the new product result the seams of which are rendered almost invisible by the hairs stuck thereover. This treatment is particularly advantageous for improving inferior quality pelts.

I claim:—

1. A method for the treatment of ready dressed and tanned pelts, consisting in painting glue solution on the hairs grown on the pelts and in brushing the hairs against the skin of the pelts.

2. A method as specified in claim 1, in which tannic substances are added to the glue solutions.

3. A method as specified in claim 1, in which fixing substances are added to the glue solutions.

PHILIPP BURGER.